

## UNITED STATES PATENT OFFICE

2,273,115

PROCESS OF PRODUCING FAST DYEINGS  
AND THE DYED FIBER OBTAINED THEREBY

Herbert Kracker, Willy Schumacher, and Vincenz Schwind, Frankfort-on-the-Main, and Wilhelm Seidenfaden, Offenbach-on-the-Main, Germany, assigns to General Aniline & Film Corporation, New York, N. Y., a corporation of Delaware

No Drawing. Application December 12, 1940,  
Serial No. 369,744. In Germany June 15, 1939

14 Claims. (Cl. 8—46)

The present invention relates to a process of producing fast dyeings and to the dyed fiber obtained thereby.

We have found that valuable dyeings of good properties of fastness are obtained on natural or artificial cellulose fibers and on animal fibers as well as on mixtures of animal fibers with cellulose fibers by applying to the material to be dyed a compound derived from 1,3,5-triazine and containing either at least one substituted or unsubstituted radical which contains an amino-group capable of being diazotized and at least one radical capable of coupling with diazo-compounds, or a radical which contains simultaneously the amino-group capable of being diazotized and the position capable of coupling with diazo-compounds, as well as at least one azo-group and a group lending solubility in water, then diazotizing the compound and causing it to combine with itself. The self-coupling may be performed or completed, for instance, by adding to the diazo-bath an agent neutralizing the acid or having an alkaline action, after the diazotization is finished, or by passing the goods through a bath having an alkaline action subsequently to the diazotization process.

The radical containing the amino-group capable of being diazotized and the radical capable of coupling with diazo-compounds may be linked to the triazine radical by a carbon-, oxygen-, nitro-  
gen- or sulfur-bond.

As radicals capable of coupling with diazo-compounds there may, for instance, be used the radicals of naphthols, of ortho-hydroxycarboxylic acids, of beta-ketocarboxylic acids, of 2-amino-5-naphthol-7-sulfonic acid, of 2-amino-8-naphthol-6-sulfonic acid, of 1-amino-8-naphthol-3,6-disulfonic acid, of 1-amino-3-dimethylaminobenzene or of pyrazolones. As further radicals the most various inorganic or organic radicals may be used.

Most of the compounds used in the present process are substantive. Owing to the substantive properties of these compounds for cellulose fibers it is possible to obtain on cellulose and regenerated cellulose as well as on mixtures of these fibers with animal fibers and, furthermore, on sheets from regenerated cellulose dyeings which are distinguished by their good properties of fastness. As far as the condensation products do not contain a sulfonic acid group, they have an affinity for cellulose esters and ethers. By treating the dyeings on the fiber with agents yielding metal their properties of fastness may be improved.

The condensation products used as parent ma-

terials may, for instance, be prepared as described in German patent specification No. 634,213.

The following examples serve to illustrate the invention, but they are not intended to limit it thereto:

(1) 1 kilo of mixed yarn consisting of 50 parts of wool and 50 parts of staple fiber from viscose is treated for 1 hour at 95° C. in a bath containing per 30 liters of water 50 grams of the 10 tertiary condensation product from cyanuric chloride, 1 mol of 2-amino-8-hydroxynaphthalene-6-sulfonic acid, 1 mol of the reduced mono-azo-dyestuff from diazotized para-nitraniline and salicylic acid and 1 mol of para-phenylenediamine, of the following formula:



and 80 grams of ammonium sulfate. 600 grams of sodium sulfate are then added and the material is further treated for half an hour at 35 80° C. It is then rinsed, diazotized in the cold for half an hour in a solution containing per 30 liters of water 25 grams of sodium nitrite, 25 grams of sodium dibutylnaphthalene sulfonate and 75 cc. of hydrochloric acid of 20° Bé. The 40 material is then treated for half an hour in a fresh bath containing per 30 liters of cold water 75 cc. of ammonia of 25 per cent strength and 5 grams of the condensation product from 1 mol of octadecylalcohol and 20 mols of ethylene-45 oxide, rinsed and dried. A brown dyeing of good properties of fastness is obtained.

When this dyeing is after-treated in the heat in an acetic acid solution with potassium bichromate, chromium fluoride or copper sulfate, 50 brown tints of an essentially improved fastness to water, to perspiration and to washing are obtained.

(2) 1 kilo of a mixture consisting of 50 parts of wool and 50 parts of staple fiber from viscose is treated for 1 hour at 95° C. in a bath con-

taining per 30 liters of water 50 grams of a condensation product of the following formula:



(obtainable by condensing cyanuric chloride with

1 mol of 2-amino-5-hydroxynaphthalene-7-sulfonic acid, 1 mol of the reduced monoazo-dyestuff from diazotized para-nitraniline and 2-amino-5-hydroxynaphthalene-7-sulfonic acid, 5 and 1 mol of para-phenylenediamine) and 80 grams of ammonium sulfate. 600 grams of sodium sulfate are then added and the material is further treated for half an hour at 80° C. It is then rinsed, diazotized and developed as described

10 in Example 1.

A red-brown dyeing of good properties of fastness is obtained. By treating the dyeing with metal salts in the heat its properties of fastness are essentially improved.

15 The following table illustrates the shades of a number of other dyeings obtainable by self-coupling according to the present invention:

|   | Parent component                                                                                                                                                                                                                                                                                                  | Shade                                                                |
|---|-------------------------------------------------------------------------------------------------------------------------------------------------------------------------------------------------------------------------------------------------------------------------------------------------------------------|----------------------------------------------------------------------|
| 1 | Condensation product from cyanuric chloride, 1 mol of 2-amino-5-hydroxynaphthalene-7-sulfonic acid, 1 mol of the reduced monoazo-dyestuff from diazotized para-nitraniline and phenol, and 1 mol of para-phenylenediamine or 1 mol of para-nitraniline with subsequent reduction, corresponding with the formula: | Subdued golden-yellow, after-treated with metal salts. orange-brown. |
| 2 |                                                                                                                                                                                                                                                                                                                   | Red-brown.                                                           |
| 3 | Condensation product from cyanuric chloride, 1 mol of 3'-aminobenzoyl-2-amino-5-hydroxynaphthalene-7-sulfonic acid, 1 mol of the reduced monoazo-dyestuff from diazotized para-nitraniline and phenol, and 1 mol of para-phenylenediamine, corresponding with the formula:                                        | Do.                                                                  |

| Parent component                                                                                                                                                                                                                                                                    | Shade                                                             |
|-------------------------------------------------------------------------------------------------------------------------------------------------------------------------------------------------------------------------------------------------------------------------------------|-------------------------------------------------------------------|
| 4 Condensation product from cyanuric chloride, 1 mol of 1-amino-8-hydroxynaphthalene-3,6-disulfonic acid, 1 mol of the reduced monoazo-dyestuff from diazotized para-nitraniline and phenol, and 1 mol of para-phenylenediamine, corresponding with the formula:                    | Yellow-brown.                                                     |
|                                                                                                                                                                                                    |                                                                   |
| 5 Condensation product from cyanuric chloride, 1 mol of 2-amino-5-hydroxynaphthalene-7-sulfonic acid, 1 mol of the reduced monoazo-dyestuff from diazotized para-nitraniline and salicylic acid, and 1 mol of para-phenylenediamine, corresponding with the formula:                | Yellow-brown, after-treated with metal salts: more yellow shade.  |
|                                                                                                                                                                                                    |                                                                   |
| 6 Condensation product from cyanuric chloride, 1 mol of 2-amino-8-hydroxynaphthalene-6-sulfonic acid, 1 mol of the reduced monoazo-dyestuff from diazotized para-nitraniline and salicylic acid, and 1 mol of para-phenylenediamine, corresponding with the formula:                | Leather-brown, after-treated with metal salts: more yellow shade. |
|                                                                                                                                                                                                  |                                                                   |
| 7 Condensation product from cyanuric chloride, 1 mol of 3-aminobenzoyl-2-amino-5-hydroxynaphthalene-7-sulfonic acid, 1 mol of the reduced monoazo-dyestuff from diazotized para-nitraniline and salicylic acid, and 1 mol of para-phenylenediamine, corresponding with the formula: | Do.                                                               |
|                                                                                                                                                                                                 |                                                                   |
| 8 Condensation product from cyanuric chloride, 1 mol of 1-amino-8-hydroxynaphthalene-3,6-disulfonic acid, 1 mol of the reduced monoazo-dyestuff from diazotized para-nitraniline and salicylic acid, and 1 mol of para-phenylenediamine, corresponding with the formula:            | Khaki-olive.                                                      |
|                                                                                                                                                                                                  |                                                                   |

|    | Parent component                                                                                                                                                                                                                                                                                                                                                                                                 | Shade         |
|----|------------------------------------------------------------------------------------------------------------------------------------------------------------------------------------------------------------------------------------------------------------------------------------------------------------------------------------------------------------------------------------------------------------------|---------------|
| 9  | Condensation product from cyanuric chloride, 1 mol of 2-amino-5-hydroxynaphthalene-7-sulfonic acid, 1 mol of the reduced monoazo-dyestuff from diazotized para-nitraniline and phenol with subsequent methylation, and 1 mol of para-phenylenediamine, corresponding with the formula:<br><br>                                 | Copper-brown. |
| 10 | Condensation product from cyanuric chloride, 1 mol of 2-amino-8-hydroxynaphthalene-6-sulfonic acid, 1 mol of the reduced monoazo-dyestuff from diazotized para-nitraniline and phenol with subsequent methylation, and 1 mol of para-phenylenediamine, corresponding with the formula:<br><br>                                 | Red-brown.    |
| 11 | Condensation product from cyanuric chloride, 1 mol of 3'-aminobenzoyl-2-amino-5-hydroxynaphthalene-7-sulfonic acid, 1 mol of the reduced monoazo-dyestuff from diazotized para-nitraniline and phenol with subsequent methylation, and 1 mol of para-phenylenediamine, corresponding with the formula:<br><br>               | Do.           |
| 12 | Condensation product from cyanuric chloride, 1 mol of 1-amino-8-hydroxynaphthalene-3,6-disulfonic acid, 1 mol of the reduced monoazo-dyestuff from diazotized para-nitraniline and phenol with subsequent methylation, and 1 mol of para-phenylenediamine, corresponding with the formula:<br><br>                           | Do.           |
| 13 | Condensation product from cyanuric chloride, 1 mol of 2-amino-5-hydroxynaphthalene-7-sulfonic acid, 1 mol of the reduced monoazo-dyestuff from diazotized para-nitraniline and 2-amino-5-hydroxynaphthalene-7-sulfonic acid in an acid solution, and 1 mol of para-phenylenediamine, corresponding with the formula:<br><br> | Do.           |

|    | Parent component                                                                                                                                                                                                                                                                                                                                                                                                                | Shade                                                                  |
|----|---------------------------------------------------------------------------------------------------------------------------------------------------------------------------------------------------------------------------------------------------------------------------------------------------------------------------------------------------------------------------------------------------------------------------------|------------------------------------------------------------------------|
| 14 | Condensation product from cyanuric chloride, 1 mol of 2-amino-8-hydroxynaphthalene-6-sulfonic acid, 1 mol of the reduced monoazo-dyestuff from diazotized para-nitraniline and 2-amino-5-hydroxynaphthalene-7-sulfonic acid in an acid solution, and 1 mol of paraphenylenediamine, corresponding with the formula:<br><br>                    | Bordeaux, after-treated with metal salts: more yellow shade.           |
| 15 | Condensation product from cyanuric chloride, 1 mol of 3'-aminobenzoyl-2-amino-5-hydroxy-naphthalene-7-sulfonic acid, 1 mol of the reduced monoazo-dyestuff from diazotized para-nitraniline and 2-amino-5-hydroxynaphthalene-7-sulfonic acid in an acid solution, and 1 mol of para-phenylenediamine, corresponding with the formula:<br><br> | Bordeaux, after-treated with metal salts: more yellow or bluer shades. |
| 16 | Condensation product from cyanuric chloride, 1 mol of 1-amino-8-hydroxynaphthalene-3,6-disulfonic acid, 1 mol of the reduced monoazo-dyestuff from diazotized para-nitraniline and 2-amino-5-hydroxynaphthalene-7-sulfonic acid in an acid solution, and 1 mol of paraphenylenediamine, corresponding with the formula:<br><br>              | Bordeaux, after-treated with metal salts: more yellow shades.          |
| 17 | The saponified condensation product from cyanuric chloride, 1 mol of 2-amino-5-hydroxynaphthalene-7-sulfonic acid, 1 mol of the reduced monoazo-dyestuff from diazotized para-nitraniline and 2-acetylamino-5-hydroxynaphthalene-7-sulfonic acid in an alkaline solution, and 1 mol of aniline, corresponding with the formula:<br><br>      | Garnet.                                                                |
| 18 | The saponified condensation product from cyanuric chloride, 1 mol of 2-amino-8-hydroxynaphthalene-6-sulfonic acid, 1 mol of the reduced monoazo-dyestuff from diazotized para-nitraniline and 2-acetylamino-5-hydroxynaphthalene-7-sulfonic acid in an alkaline solution, and 1 mol of aniline, corresponding with the formula:<br><br>      | Intense garnet.                                                        |

|    | Parent component                                                                                                                                                                                                                                                                                                                                   | Shade             |
|----|----------------------------------------------------------------------------------------------------------------------------------------------------------------------------------------------------------------------------------------------------------------------------------------------------------------------------------------------------|-------------------|
| 19 | The saponified condensation product from cyanuric chloride, 1 mol of 3'-aminobenzoyl-2-amino-5-hydroxy-naphthalene-7-sulfonic acid, 1 mol of the reduced monoazo-dyestuff from diazotized para-nitraniline and 2-acetylaminio-5-hydroxy-naphthalene-7-sulfonic acid in an alkaline solution, and 1 mol of aniline, corresponding with the formula: | Violetish garnet. |
|    |                                                                                                                                                                                                                                                                                                                                                    |                   |
| 20 | The saponified condensation product from cyanuric chloride, 1 mol of 1-amino-8-hydroxynaphthalene-3,6-disulfonic acid, 1 mol of the reduced monoazo-dyestuff from diazotized para-nitraniline and 2-acetylaminio-5-hydroxynaphthalene-7-sulfonic acid in an alkaline solution, and 1 mol of aniline, corresponding with the formula:               | Dark garnet.      |
|    |                                                                                                                                                                                                                                                                                                                                                    |                   |
| 21 | The reduced condensation product from cyanuric chloride, 1 mol of 2-amino-5-hydroxy-naphthalene-7-sulfonic acid, 1 mol of the monoazo-dyestuff from diazotized para-nitraniline and aminohydroquinonedimethylether, and 1 mol of aniline, corresponding with the formula:                                                                          | Current.          |
|    |                                                                                                                                                                                                                                                                                                                                                    |                   |
| 22 | The reduced condensation product from cyanuric chloride, 1 mol of 2-amino-8-hydroxynaphthalene-6-sulfonic acid, 1 mol of the monoazo-dyestuff from diazotized para-nitraniline and aminohydroquinonedimethylether, and 1 mol of aniline, corresponding with the formula:                                                                           | Red-brown.        |
|    |                                                                                                                                                                                                                                                                                                                                                    |                   |
| 23 | The reduced condensation product from cyanuric chloride, 1 mol of 3'-aminobenzoyl-2-amino-5-hydroxy-naphthalene-7-sulfonic acid, 1 mol of the monoazo-dyestuff from diazotized para-nitraniline and aminohydroquinonedimethylether, and 1 mol of aniline, corresponding with the formula:                                                          | Do.               |
|    |                                                                                                                                                                                                                                                                                                                                                    |                   |
| 24 | The reduced condensation product from cyanuric chloride, 1 mol of 1-amino-8-hydroxynaphthalene-3,6-disulfonic acid, 1 mol of the monoazodyestuff from diazotized para-nitraniline and aminohydroquinonedimethylether, and 1 mol of aniline, corresponding with the formula:                                                                        | Brown.            |
|    |                                                                                                                                                                                                                                                                                                                                                    |                   |

|    | Parent component                                                                                                                                                                                                                                                                                                            | Shade                |
|----|-----------------------------------------------------------------------------------------------------------------------------------------------------------------------------------------------------------------------------------------------------------------------------------------------------------------------------|----------------------|
| 25 | The reduced condensation product from cyanuric chloride, 1 mol of 2-amino-5-hydroxynaphthalene-7-sulfonic acid, 1 mol of the monoazo-dyestuff from diazotized para-nitraniline and 2-amino-5-hydroxynaphthalene-7-sulfonic acid in an alkaline medium, and 1 mol of aniline, corresponding with the formula:                | Brown.               |
|    |                                                                                                                                                                                                                                                                                                                             |                      |
| 26 | The reduced condensation product from cyanuric chloride, 1 mol of 2-amino-8-hydroxynaphthalene-6-sulfonic acid, 1 mol of the monoazo-dyestuff from diazotized para-nitraniline and 2-amino-8-hydroxynaphthalene-7-sulfonic acid in an alkaline medium, and 1 mol of aniline, corresponding with the formula:                | Dark garnet.         |
|    |                                                                                                                                                                                                                                                                                                                             |                      |
| 27 | The reduced condensation product from cyanuric chloride, 1 mol of 3'-aminobenzoyl-2-amino-5-hydroxynaphthalene-7-sulfonic acid, 1 mol of the monoazo-dyestuff from diazotized paranitraniline and 2-amino-5-hydroxynaphthalene-7-sulfonic acid in an alkaline medium, and 1 mol of aniline, corresponding with the formula: | Violetish dark-blue. |
|    |                                                                                                                                                                                                                                                                                                                             |                      |
| 28 | The reduced condensation product from cyanuric chloride, 1 mol of 1-amino-8-hydroxynaphthalene-3,6-disulfonic acid, 1 mol of the monoazo-dyestuff from diazotized para-nitraniline and 2-amino-5-hydroxynaphthalene-7-sulfonic acid in an alkaline medium, and 1 mol of aniline, corresponding with the formula:            | Bordeaux-garnet.     |
|    |                                                                                                                                                                                                                                                                                                                             |                      |
| 29 | The reduced condensation product from cyanuric chloride, 1 mol of 2-amino-5-hydroxynaphthalene-7-sulfonic acid, 1 mol of the monoazo-dyestuff from diazotized 2-chloro-4-nitraniline and 2-amino-5-hydroxynaphthalene-7-sulfonic acid in an alkaline medium, and 1 mol of aniline, corresponding with the formula:          | Currant.             |
|    |                                                                                                                                                                                                                                                                                                                             |                      |
| 30 | The reduced condensation product from cyanuric chloride, 1 mol of 1-amino-8-hydroxynaphthalene-3,6-disulfonic acid, 1 mol of the monoazo-dyestuff from diazotized 2-chloro-4-nitraniline and 2-amino-5-hydroxynaphthalene-7-sulfonic acid in an alkaline medium, and 1 mol of aniline, corresponding with the formula:      | Garnet.              |
|    |                                                                                                                                                                                                                                                                                                                             |                      |

|    | Parent component                                                                                                                                                                                                                                                                                                                                                                                                  | Shade            |
|----|-------------------------------------------------------------------------------------------------------------------------------------------------------------------------------------------------------------------------------------------------------------------------------------------------------------------------------------------------------------------------------------------------------------------|------------------|
| 31 | The reduced condensation product from cyanuric chloride, 1 mol of 1-amino-8-hydroxynaphthalene-3,6-disulfonic acid, 1 mol of the reduced monoazo-dyestuff from diazotized para-nitraniline and salicylic acid, and 1 mol of the monoazo-dyestuff from diazotized 2-methyl-5-methoxy-4-nitraniline and 1-amino-8-hydroxynaphthalene-3,6-disulfonic acid in an alkaline medium, corresponding with the formula:<br> | Garnet.          |
| 32 | The saponified condensation product from cyanuric chloride, 1 mol of 2-amino-5-hydroxynaphthalene-7-sulfonic acid, 1 mol of the reduced monoazo-dyestuff from diazotized 2-chloro-4-nitraniline and 2-acetyl-amino-5-hydroxynaphthalene-7-sulfonic acid in an alkaline medium, and 1 mol of aniline, corresponding with the formula:<br>                                                                          | Dark garnet.     |
| 33 | The saponified condensation product from cyanuric chloride, 1 mol of 3'-aminobenzoyl-2-amino-5-hydroxynaphthalene-7-sulfonic acid, 1 mol of the reduced monoazo-dyestuff from diazotized 2-chloro-4-nitraniline and 2-acetyl-amino-5-hydroxynaphthalene-7-sulfonic acid in an alkaline medium, and 1 mol of aniline, corresponding with the formula:<br>                                                          | Dark violet.     |
| 34 | Condensation product from cyanuric chloride, 1 mol of 1-(4'-aminophenyl)-3-methyl-5-pyrazolone, 1 mol of 2,6-dichloro-1,4-diaminobenzene and 1 mol of 4-amino-1,1'-azobenzene-4'-sulfonic acid, corresponding with the formula:<br>                                                                                                                                                                               | Reddish yellow.  |
| 35 | Condensation product from cyanuric chloride, 1 mol of 1-(3'-aminophenyl)-5-pyrazolone-3-carboxylic acid, 1 mol of 2,6-dichloro-1,4-diaminobenzene and 1 mol of 4-amino-1,1'-azobenzene-4'-sulfonic acid, corresponding with the formula:<br>                                                                                                                                                                      | Brownish yellow. |

|    | Parent component                                                                                                                                                                                                                                                                      | Shade             |
|----|---------------------------------------------------------------------------------------------------------------------------------------------------------------------------------------------------------------------------------------------------------------------------------------|-------------------|
| 36 | Condensation product from cyanuric chloride, 1 mol of 2-amino-5-hydroxynaphthalene-7-sulfonic acid, 1 mol of 2,6-dichloro-1,4-diaminobenzene and 1 mol of 4-amino-1,1'-azobenzene-4'-sulfonic acid, corresponding with the formula:<br><br>                                           | Yellowish red.    |
| 37 | Condensation product from cyanuric chloride, 1 mol of 2-amino-5-hydroxynaphthalene-7-sulfonic acid and 1 mol of 4,4'-diamino-2-methyl-5-methoxy-1,1'-azobenzene, corresponding with the probable formula:<br><br>                                                                     | Dark brown.       |
| 38 | Condensation product from cyanuric chloride, 1 mol of 1-amino-5-hydroxynaphthalene-7-sulfonic acid, 1 mol of 4,4'-diamino-2-methyl-5-methoxy-1,1'-azobenzene and 1 mol of 1-aminobenzene-4-sulfonic acid, corresponding with the probable formula:<br><br>                            | Intense currant.  |
| 39 | Condensation product from cyanuric chloride, 1 mol of 2-amino-5-hydroxynaphthalene-7-sulfonic acid, 1 mol of 2,6-dichloro-1,4-diaminobenzene and 1 mol of the reduced monoazo-dye stuff from diazotized para-nitroaniline and salicylic acid, corresponding with the formula:<br><br> | Middle red-brown. |
| 40 | Condensation product from cyanuric chloride, 1 mol of 1-amino-8-hydroxynaphthalene-4-sulfonic acid and 1 mol of 4,4'-diamino-2-methyl-5-methoxy-1,1'-azobenzene, corresponding with the probable formula:<br><br>                                                                     | Reddish brown.    |

|    | I parent component                                                                                                                                                                                                                                                                  | Shade                    |
|----|-------------------------------------------------------------------------------------------------------------------------------------------------------------------------------------------------------------------------------------------------------------------------------------|--------------------------|
| 41 | Condensation product from cyanuric chloride, 1 mol of 1-amino-8-hydroxynaphthalene-4-sulfonic acid, 1 mol of 2,6-dichloro-1,4-diaminobenzene and 1 mol of the reduced monoazo-dyestuff from diazotized para-nitraniline and salicylic acid, corresponding with the formula:<br><br> | Yellowish brown.         |
| 42 | Condensation product from cyanuric chloride, 1 mol of 1-amino-5-hydroxynaphthalene-7-sulfonic acid, 1 mol of 2,6-dichloro-1,4-diaminobenzene and 1 mol of the reduced monoazo-dyestuff from diazotized para-nitraniline and salicylic acid, corresponding with the formula:<br><br> | Intensely reddish brown. |
| 43 | Condensation product from cyanuric chloride, 1 mol of 1-amino-8-hydroxynaphthalene-5-sulfonic acid and 1 mol of 4,4'-diamino-2-methyl-5-methoxy-1,1'-azobenzene, corresponding with the probable formula:<br><br>                                                                   | Reddish brown.           |
| 44 | Condensation product from cyanuric chloride, 1 mol of 1-amino-8-hydroxynaphthalene-5-sulfonic acid, 1 mol of 2,6-dichloro-1,4-diaminobenzene and 1 mol of the reduced monoazo-dyestuff from diazotized para-nitraniline and salicylic acid, corresponding with the formula:<br><br> | Brown.                   |

|    | Parent component                                                                                                                                                                                                                                                           | Shade            |
|----|----------------------------------------------------------------------------------------------------------------------------------------------------------------------------------------------------------------------------------------------------------------------------|------------------|
| 45 | Condensation product from cyanuric chloride, 1 mol of 2-amino-8-hydroxynaphthalene-6-sulfonic acid, 1 mol of 4,4'-diamino-2-methyl-5-methoxy-1,1'-azobenzene and 1 mol of 1-aminobenzene-4-sulfonic acid, corresponding with the probable formula:                         | Intense currant. |
|    |                                                                                                                                                                                           |                  |
| 46 | Condensation product from cyanuric chloride, 1 mol of 2-amino-8-hydroxynaphthalene-6-sulfonic acid, 1 mol of 4-amino-1,1'-azobenzene-4'-sulfonic acid and 1 mol of 2,6-dichloro-1,4-diaminobenzene, corresponding with the formula:                                        | Brownish red.    |
|    |                                                                                                                                                                                          |                  |
| 47 | Condensation product from cyanuric chloride, 1 mol of 2-amino-8-hydroxynaphthalene-6-sulfonic acid, 1 mol of 2,6-dichloro-1,4-diaminobenzene and 1 mol of the reduced monoazo-dyestuff from diazotized paranitraniline and salicylic acid, corresponding with the formula: | Yellow-brown.    |
|    |                                                                                                                                                                                         |                  |

We claim:

1. Process of producing fast dyeings on fibrous material of the group consisting of cellulose fibers, animal fibers and mixtures of animal fibers with cellulose fibers, which comprises applying to the fiber a compound derived from 1,3,5-triazine containing an azo group, a group conferring solubility in water, a diazotizable amino group and a grouping which is capable of coupling with a diazo compound, then diazotizing the compound on the fiber and causing self-coupling by an alkaline treatment.

2. Process of producing fast brown dyeings on fibrous material of the group consisting of cellulose fibers, animal fibers and mixtures of animal fibers with cellulose fibers, which comprises applying to the fiber the condensation product from cyanuric chloride, 1 mol of 2-amino-8-hydroxynaphthalene-6-sulfonic acid, 1 mol of the reduced monoazo-dyestuff from diazotized para-nitraniline and salicylic acid and 1 mol of para-

55 phenylenediamine, corresponding with the formula:



then diazotizing the compound on the fiber and causing self-coupling by an alkaline treatment.

3. Process of producing fast brown dyeings on fibrous material of the group consisting of cellulose fibers, animal fibers and mixtures of animal fibers with cellulose fibers, which comprises applying to the fiber the condensation product from

cyanuric chloride, 1 mol of 2-amino-8-hydroxynaphthalene-6-sulfonic acid, 1 mol of the reduced monoazo-dyestuff from diazotized para-nitraniline and salicyclic acid and 1 mol of para-phenylenediamine, corresponding with the formula:



then diazotizing the compound on the fiber, causing self-coupling by an alkaline treatment and treating the dyeing with an agent yielding metal.

4. Process of producing fast red-brown dyeings on fibrous material of the group consisting of cellulose fibers, animal fibers and mixtures of animal fibers with cellulose fibers, which comprises applying to the fiber the condensation product from cyanuric chloride, 1 mol of 2-amino-8-hydroxynaphthalene-6-sulfonic acid, 1 mol of the reduced monoazo-dyestuff from diazotized para-nitraniline and phenol, and 1 mol of para-phenylenediamine, corresponding with the formula:



then diazotizing the compound on the fiber and causing self-coupling by an alkaline treatment.

5. Process of producing fast red-brown dyeings on fibrous material of the group consisting of cellulose fibers, animal fibers and mixtures of animal fibers with cellulose fibers, which comprises applying to the fiber the condensation product from cyanuric chloride, 1 mol of 2-amino-8-hydroxynaphthalene-6-sulfonic acid, 1 mol of the reduced monoazo-dyestuff from diazotized para-nitraniline and phenol, and 1 mol of para-phenylenediamine, corresponding with the formula:



then diazotizing the compound on the fiber, causing self-coupling by an alkaline treatment and

treating the dyeing with an agent yielding metal.

6. Process of producing fast leather-brown dyeings on fibrous material of the group consisting of cellulose fibers, animal fibers and mixtures of animal fibers with cellulose fibers, which comprises applying to the fiber the condensation product from cyanuric chloride, 1 mol of 2-amino-8-hydroxynaphthalene-6-sulfonic acid, 1 mol of the reduced monoazo-dyestuff from diazotized para-nitraniline and salicyclic acid, and 1 mol of para-phenylenediamine, corresponding with the formula:



then diazotizing the compound on the fiber and causing self-coupling by an alkaline treatment.

7. Process of producing fast leather-brown dyeings on fibrous material of the group consisting of cellulose fibers, animal fibers and mixtures of animal fibers with cellulose fibers, which comprises applying to the fiber the condensation product from cyanuric chloride, 1 mol of 2-amino-8-hydroxynaphthalene-6-sulfonic acid, 1 mol of the reduced monoazo-dyestuff from diazotized para-nitraniline and salicyclic acid, and 1 mol of para-phenylenediamine, corresponding with the formula:



then diazotizing the compound on the fiber, causing self-coupling by an alkaline treatment and treating the dyeing with an agent yielding metal.

8. Fiber dyed with an azo-compound obtainable on the fiber by the process claimed in claim 1.

9. Fiber dyed with an azo-compound obtainable on the fiber by the process claimed in claim 2.

10. Fiber dyed with an azo-compound obtainable on the fiber by the process claimed in claim 3.

11. Fiber dyed with an azo-compound obtainable on the fiber by the process claimed in claim 4.

12. Fiber dyed with an azo-compound obtainable on the fiber by the process claimed in claim 5.

13. Fiber dyed with an azo-compound obtainable on the fiber by the process claimed in claim 6.

14. Fiber dyed with an azo-compound obtainable on the fiber by the process claimed in claim 7.

HERBERT KRACKER.  
WILLY SCHUMACHER.  
VINZENZ SCHWIND.  
WILHELM SEIDENFADEN.